

Dec. 18, 1956

C. L. NOTTEBOHM ET AL  
PROCESS FOR THE MANUFACTURE OF POROUS  
FLEXIBLE SHEET MATERIAL  
Filed Sept. 1, 1953

2,774,687



INVENTORS:

CARL LUDWIG NOTTEBOHM  
WERNER JACOB  
WILHELM LAUPPE  
ROBERT SCHIBERT

By  
Richardson, David and Verlin

ATTORNEYS.

1

2,774,687

## PROCESS FOR THE MANUFACTURE OF POROUS FLEXIBLE SHEET MATERIAL

Carl Ludwig Nottebohm, Weinheim an der Bergstrasse, Germany, Werner Jacob, Lowell, Mass., and Wilhelm Lauppe and Robert Schabert, Weinheim an der Bergstrasse, Germany

Application September 1, 1953, Serial No. 377,979

Claims priority, application Germany September 3, 1952

9 Claims. (Cl. 117—120)

The present invention relates to the manufacture of porous, flexible sheet material similar to textile or leather which involves impregnating fiber fleeces with film-forming binders, preferably emulsions or dispersions of natural and/or synthetic rubber and solidification of the impregnated material by subsequent steps, such as drying or treatment with coagulating or precipitating agents and, if necessary, vulcanization and/or hardening.

Certain processes of this type are described and claimed in Patent Nos. 2,719,806, 2,719,802 and 2,719,795, all filed December 22, 1951, and issued October 4, 1955. As described in these applications, the starting material for processes of the type in question may consist of fibers or fiber mixtures of various types and compositions. As examples, may be mentioned vegetable fibers, such as cotton, ramie, flax, jute, animal fibers, such as wool and other animal hair or human hair, or synthetic fibers, such as viscose fibers, acetate fibers, superpolyamide fibers, polyvinyl fibers, polyvinylidene fibers, polyethylene fibers, polyester fibers, polyacryl fibers, fibers consisting of copolymers of several fiber-forming monomeric compounds, protein fibers, alginate fibers, casein fibers, mineral fibers, such as glass- or stone-wool or asbestos fibers, or mixtures of two or more of the above mentioned types of fibers. It is essential that the fibers are used in cardable form. Their length should be generally about 0.8 to 8 cm., preferably about 2 to 6 cm. Fibers such as horse-hair, cocoanut fibers, etc. which are too long or too thick and which have hard and smooth surfaces, rendering them unsuitable for carding on ordinary carding machines have generally been found unsuitable for use in processes of the type in question.

Suitable binders are, as mentioned heretofore, preferably emulsions or dispersions of natural and/or synthetic rubber. Excellent results have been obtained, for instance, with polymers of butadiene-acrylonitrile, butadiene-styrene, their derivatives, such as chloroprene, and their copolymers. The emulsions or dispersions used for impregnating the fiber fleece may contain one or more additional components, such as wetting agents, dispersing agents, thickening agents, antioxidants, fillers, vulcanizing agents, vulcanization accelerators and the like. The aqueous emulsions or dispersions may contain about 15 to 35% by weight and preferably about 20 to 29% by weight of solid binder, such as natural rubber. Wetting agents, such as sodium isobutylene naphthylene sulphonate (Nekal) may be present in an amount up to 60% by weight of the solid binder content of the dispersion. Preferably about 20 to 28 parts by solid weight of wetting agents are used for each 100 parts by weight of binder solids. The antioxidants used are those commonly employed in the rubber industry, such as, for instance, para-phenylenediamine derivatives, mercapto benzimidazol or

2

phenyl beta-naphthylamine. A preferred method of manufacturing fibrous sheet material, as described in the above mentioned copending applications comprises the following steps:

5 The fibers or fiber mixtures, which may first have been pretreated by washing or boiling and drying, are formed on a carding machine into thin, loose, fibrous webs having a weight of about 15 to 35 g. per square meter. A number of such webs, for instance 3 to 20, are placed 10 upon one another and subjected to a suitable pressure to produce fleeces of the desired thickness which may have a weight of about 40 to 400 g. or more per square meter. In order to give to the fleeces equal resistance against stresses in the longitudinal direction and in the transverse direction, the thin webs, the fibers of which have been partially aligned in longitudinal direction by the carding operation, are placed upon one another at an angle in such a manner that the fibers of adjacent layers cross each other and, thus, a fleece is formed in which 15 the fibers extend in various directions, i. e., the fibers are polypersed. In order to obtain an intimate cohesion between the superposed webs and to produce a light felting, increased denseness and smooth surfaces, the multi-layer fleeces are passed through pressure rollers heated to about 20 60 to 80° C.

The resulting, unstable fleeces are subjected to a surface treatment, which consists in the application of a small quantity of binder liquid to one surface of the fleece, for instance, by spraying or by means of rollers. 25 Advantageously the binder liquid is spread on the surface of the fleece in the form of a stiff foam having a high air content. When the fleece is dried, its surface fibers are cemented together at their crossing points under preservation of practically all the interstices between 30 the fibers and the surface of the fleece is coated with a thin, spider-web like net of binder. This unilateral surface treatment stabilizes the fleece sufficiently to permit its through impregnation, for instance by passing it through roller pairs, without danger of the fleece being torn or seriously distorted.

The unilaterally stabilized fleece is now through impregnated by passing it through a pair of rollers having their axes disposed in a horizontal plane while a suitable film-forming binder liquid is pressed through its untreated surface uniformly in such a manner that it penetrates the entire thickness of the fleece. The binder liquid is preferably used in the through impregnating step in the form of a stable, flowable foam.

The impregnated fleece or sheet material is dried for instance, by passing it through a drying chamber heated to about 80 to 120° C. This drying step may also involve a vulcanization or final vulcanization of the rubber binder.

After drying, the material may be subjected to the usual after-treatments, such as calendering, washing, etc. Subsequent to calendering, final vulcanization may be effected, for instance, by heating the material to temperatures of 100° C. or higher. Dependent upon the type and composition of the fibrous material, the type and composition of the binder, the quantity proportions between fibrous material and binder and the specific conditions under which the impregnation is carried out, products can be obtained which have the properties desired for the particular purpose for which the material is intended, such as softness, porosity, elasticity, springiness, crease-resistance, water resistance, and fastness against washing and cleaning. The material may also be treated in such away that it can be stitched, padded or sewed on

sewing machines, and it can be dyed any desired color.

The quantity of the film-forming binder material introduced into the fiber fleece is, preferably, so selected that the fibers are cemented together at their crossing points only and such interstices or pores are maintained that porous structures are formed which are similar to textiles. Generally, it has been found advantageous to produce sheet material containing about 25 to about 65 percent by weight and (preferably about 35 to 55% by weight) of solid binder particles and about 75 to 35% by weight of fibrous material. The finished sheet material has a thickness of about 0.15 to 1.5 millimeter and, preferably, of about 0.2 to 0.9 millimeter. It is soft, flexible and has a textile-like feel and drape, uniform porosity and excellent elasticity. As compared to ordinary textile fabrics, which have different properties in the direction of the woof and of the warp, sheet materials prepared by the described process are distinguished by iso-elasticity; that is, they are resiliently and uniformly resistant to creasing or folding in any direction.

If the described process is used for the manufacture of form-giving and form-retaining interlinings or stiffening materials or as cold and dust protecting interlinings for clothing, it is preferred to use fiber fleeces which contain wool, possibly mixed with other fibers and to treat such fleeces with aqueous dispersions or emulsions of natural or synthetic rubber containing vulcanizing agents, vulcanization accelerators, wetting agents and anti-oxidants. After impregnation, the products are vulcanized, then freed of water-soluble components by washing and finally dried. The fiber fleeces used for these purposes should generally contain at least 15% by weight, and preferably from 20 to 70% by weight, of wool fibers.

Binder liquids which are preferred for use in the described process are emulsions or dispersions of synthetic rubbers or mixtures thereof, the Defo values of which in dry condition are between 1000 and 8000 degrees Defo. As will be understood by those familiar with the art, the term "Defo hardness" designates the force in grams which is required to compress a rubber test cylinder of 10 millimeter height and 10 millimeter diameter at 80° C. in thirty seconds by 4 millimeter (compare Houwink, page 450). The Defo values determine the degree of softness and the degree of elasticity of the rubber.

For the preparation of softer, still fabric-like products of less springiness, fiber mixtures may be used which do not contain any wool fibers. Thus, a fleece made from a mixture of 30 parts by weight of polyamide fiber, 30 parts by weight of cell wool acetate fiber, 20 parts by weight of ramie fiber combings and 20 parts by weight of cell wool viscose fiber may be impregnated with a soft, synthetic rubber (Defo value between about 800 and 1700).

In some cases it is advantageous to incorporate into the fibrous sheet material water repellent lubricants, such as paraffin, wax or the like in quantities of about 2 to 10% by weight. These materials act during sewing, especially sewing on sewing machines, as lubricants for the needles. The water repellent lubricants can be used in combination with other water repellent materials, such as aluminum salts; preferably the water repellent lubricants or other water repellents are incorporated into the solidified and vulcanized sheet material after washing thereof.

While the products obtainable by the heretofore described methods, as particularly set forth and disclosed in the applicant's above mentioned copending patent applications, produce valuable sheet material having outstanding properties with regard to porosity, elasticity, springiness, etc., it has now been found that the products can be further improved, particularly as regards their springiness, their fastness against dry cleaning and their abrasion resistance. It is the principal object of

the present invention to provide methods for attaining such improvements.

In order to accomplish this object, it is proposed, according to the present invention, to incorporate into the fiber fleeces in addition to the above mentioned film-forming binders and previously specified additional components, such as vulcanizing agents, vulcanization accelerators, fillers, water repellants, etc., certain relatively small quantities of synthetic resin condensates. Suitable synthetic resin condensates are, for instance, condensates of aldehydes, and preferably condensates of formaldehyde with substances which can be condensed with aldehydes, such as phenols and derivatives thereof, urea and urea compounds and derivatives, such as cyanamide, dicyandiamide, melamine, etc. Generally, such poly-condensates may be used which, in their final poly-condensed condition, are insoluble in water and inert against organic solvents of the type used, for instance, in the dry cleaning of clothing and the like.

According to a preferred embodiment of the present invention, the superpoly-condensates are incorporated into the fibrous products advantageously in the form of their pre-condensates which are still soluble in water. Such water soluble pre-condensate may, for instance, be admixed to a rubber dispersion or emulsion which may also contain other components, such as wetting agents, vulcanizing agents, vulcanization accelerators and the like, and this mixture may be used for the through impregnation of the fiber fleeces. It is preferred to incorporate into the aqueous mixture additional substances which are capable of promoting or accelerating the conversion of the condensation products to their insoluble final state. Suitable condensation activators are, for instance, alkali compositions, such as caustic soda solution, earth alkali compositions, such as barium chloride, ammonium salts, such as ammonium chloride, organic acids, such as lactic acid and sulphonic acids or their salts, such as sodium lauryl sulphonate or soaps of the type obtainable from fatty acids plus ammonia. Sometimes, certain components of the impregnating dispersion which are present for other purposes, such as vulcanizing agents, vulcanization accelerators, anti-oxidants or emulsifying agents may act as condensation activators. A material which can serve such double purpose is, for instance, hexamethylene tetramine.

The most suitable quantities of poly-condensates to be used can be ascertained by simple tests and range from about 1-15% by weight of the binder solids. In the manufacture of sheet material which is intended as interlining for articles of clothing, the quantities of poly-condensates to be employed may be determined on the basis of the Defo values of the rubbers used in the binder liquids, as shown by the following table:

| Defo values of Rubber | Parts by Weight of Polycondensate per 100 Parts by Weight of Rubber (solid) |
|-----------------------|-----------------------------------------------------------------------------|
| 1,000                 | 6 to 8                                                                      |
| 1,250                 | 4 to 6                                                                      |
| 4,500                 | 2 to 4                                                                      |
| 8,000                 | 1 to 2                                                                      |

It has been found desirable to use the dispersions or emulsions which, according to the invention, contain, in addition to the rubber binders, also water soluble pre-condensates of synthetic resins, such as precondensates of formaldehyde with phenols, urea and the like, in the form of a foam, in the manner described and claimed in applicant's co-pending U. S. patent applications 262,941 and 262,942 mentioned above. Accordingly, care must be taken to introduce the synthetic resin precondensates in such a manner and quantity into the impregnating binder dispersion that they do not prevent the conversion of the dispersion into a stable foam suitable for

impregnation of the fleeces. For this reason, generally, according to the invention, only relatively small quantities of water soluble precondensates of water soluble compounds capable of condensation are added to the impregnating dispersions. In some cases, it has also been found advantageous to incorporate into the fibrous fleeces or into the impregnating dispersions, softening agents of the type generally used in the synthetic resin condensate industry. Typical softening agents of this type are, for instance, glycerine, glycols, fatty acid esters and the like.

The impregnation of the fiber fleeces may be carried out in the manner described above and set forth in detail in the applicant's above mentioned co-pending applications by converting the impregnating dispersion containing, in addition to the film-forming binders, also precondensates of synthetic resins, such as formaldehyde with substances condensable therewith, and possibly other desired components, to a stable, flowable foam and pressing this foam by means of rollers into the fleeces. The stabilization of the impregnation may be effected by heat agglomeration such as, for instance, simple drying. For this purpose, the impregnated fleeces may be passed through heating chambers. Care must be taken to carry out the after-treatment of the impregnated fleeces under such conditions that the precondensates are converted to their water insoluble and solvent resistant final form. In order to accomplish this result, the drying and vulcanization steps may be suitably modified with regard to the temperature and the duration of the heat treatment. According to one embodiment of the process according to the invention, the impregnated sheet material is subjected, after heat coagulation, to a vulcanizing treatment at temperatures from about 80 to 120° C. which is continued until complete vulcanization of the rubber and simultaneous complete conversion of the synthetic resin condensate to its final condensed state has taken place. Thereafter, the material may be washed and subjected to any other desired after treatment.

The vulcanization and hardening of the synthetic resin condensates may also be carried out in several stages. Thus, the impregnated and dried material may first be prevulcanized at temperatures of 80 to 95° C., then calendered, washed and passed through a paraffin emulsion bath. Thereafter, the rubber components may be finally vulcanized and the synthetic resin condensates may be converted to their final insoluble state or hardened by subjecting the impregnated sheet material for about 24 hours to temperatures between 80° to 100° C. It will be understood that the heat treatments must be carried out under such conditions that the fibers are not damaged. Generally, it is recommended to use temperatures not exceeding about 135° C.

Due to the incorporation of hardened condensation products of aldehydes, preferably formaldehyde, with substances which can be condensed therewith, such as phenols, ureas, etc., the properties of the products according to the invention are improved in various respects. Thus, the incorporation into a fiber fleece of a quantity of phenol formaldehyde condensate in an amount of about 4% by weight of the film forming elastic rubber solids constituting the primary binder leads to products having substantially improved springiness and abrasion resistance. Such products are particularly suitable for use as interlinings in clothing.

The accompanying drawing shows several alternate procedures in accordance with the present invention.

The following examples may serve to illustrate the invention.

#### Example 1

A fiber mixture consisting of 30 parts by weight of cotton combings, 30 parts by weight of ramie combings and 40 parts by weight of cell wool combings was formed into a fiber fleece having a weight of 135 g. per square

millimeter. The fleece was condensed and stretched between pressure rollers heated to 80° C.

A stiff foam was formed from an aqueous dispersion of the following composition:

|                                                                | Liquid<br>Parts<br>B. W. | Solid<br>Parts<br>B. W. |
|----------------------------------------------------------------|--------------------------|-------------------------|
| 10 Butadiene-acrylonitrile polymer dispersion (37%)            | 270                      | 100                     |
| Sodiumbenzenesulphonate solution (40%)                         | 67.5                     | 27                      |
| Sulphur dispersion (80%)                                       | 3.75                     | 3                       |
| Zincoxide dispersion (50%)                                     | 10                       | 5                       |
| Zinc salt of phenylethyldithiocarbaminic acid dispersion (25%) | 4                        | 1                       |
| Softened water                                                 | 442                      | -----                   |

15

The foam was spread uniformly in a very thin layer by means of a doctor blade onto one surface of the fiber fleece while the fleece was passed under the blade, whereupon the fleece was dried.

20

The sheet material, stabilized by this unilateral pre-treatment, was now passed between a pair of cooperating rollers with smooth surfaces having their axes arranged in a horizontal plane, and a stable, flowable aqueous foam was pressed into the fleece through its untreated surface, so as to penetrate the cutive thickness of the fleece. The foam was prepared from a dispersion of the following composition:

|                                                                | Liquid<br>Parts<br>B. W. | Solid<br>Parts<br>B. W. |
|----------------------------------------------------------------|--------------------------|-------------------------|
| 30 Butadiene Acrylonitrile dispersion (35%)                    | 244                      | 95                      |
| Phenol-formaldehyde precondensate solution (65%)               | 9.10                     | 5                       |
| Sulphur dispersion (50%)                                       | 4                        | 2                       |
| Zincoxide dispersion (40%)                                     | 125                      | 5                       |
| Zinc salt of phenylethyldithiocarbaminic acid dispersion (25%) | 6                        | 1.5                     |
| Paraphenyldiamine derivative solution (25%)                    | 6                        | 1.5                     |
| Sodiumsulphate                                                 | 116                      | 16                      |
| Softened water                                                 | -----                    | -----                   |

40

The mixture contained about 22.5% by weight of the solution of rubber solids and about 25.2% by weight of the solution of total solids.

45

The impregnated fleece was now passed through a drying chamber where it was dried at about 90 to 100° C. for twenty minutes and simultaneously pre-vulcanized. The resulting highly porous sheet material, which already exhibited good springiness, was now finally vulcanized and hardened for about twenty-four hours at 75° C. in a drying chamber. Thereafter, it was washed in a washing machine in the manner customary in the textile industry whereby all water soluble substances were dissolved out. Then, the material was dried again and treated with paraffin-wax-aluminum salt dispersion to make it water repellent. The final product had a thickness of .8 to 1 millimeter and a weight of about 220 g. per square millimeter. Its rubber content was about 42% by weight. The material had the particular advantage that its properties were not significantly impaired by dry cleaning. It exhibited excellent springiness after dry cleaning.

50

#### Example 2

65 A mixture of 50 parts by weight of cotton combings and 50 parts by weight of cell wool was formed into thin fibrous webs and a number of these webs were superposed upon one another to produce a fleece containing fibers disposed in all directions and having, after stretching, a weight of about 70 to 100 g. per square meter. One surface of the fleece was pretreated with a foam having the same composition as the pretreatment foam described in Example 1.

60

After drying, the unilaterally prestablized fleece was treated by means of a pair of rollers, as described in Ex-

70

ample 1, with a stable, flowable foam obtained from a dispersion of the following composition:

|                                                                 | Liquid<br>Parts<br>B. W. | Solid<br>Parts<br>B. W. |
|-----------------------------------------------------------------|--------------------------|-------------------------|
| Butadienestyrene polymer dispersion (40%)                       | 125                      | 50                      |
| Butadiene-acrylonitrile polymer dispersion (60%)                | 83.5                     | 50                      |
| Phenylformaldehyde precondensate solution (50%)                 | 5                        | 2.5                     |
| Sodiumbenzenesulphonate solution (67.5%)                        | 30                       | 20                      |
| Sulphur dispersion (80%)                                        | 3.75                     | 3                       |
| Zincoxide dispersion (50%)                                      | 10                       | 5                       |
| Zinc salt of phenylethyldithiocarbamic acid as dispersion (25%) | 4                        | 1.5                     |
| Paraphenylenediamine derivative (25%)                           | 8                        | 2                       |
| Softened water                                                  | 418                      | -----                   |

The impregnated material was treated with a saturated sodiumsulphate solution and dried. Thereafter, it was subjected to a second impregnation by passing the sheet material through a pair of rollers with smooth surfaces and pressing into both surfaces of the sheet an aqueous paste of the following composition:

|                                                                 | Liquid<br>Parts<br>B. W. | Solid<br>Parts<br>B. W. |
|-----------------------------------------------------------------|--------------------------|-------------------------|
| Butadiene-acrylonitrile dispersion (37%)                        | 270                      | 100                     |
| Starch solution (35%)                                           | 275                      | 90                      |
| Sodiumsulphate                                                  |                          | 100                     |
| Sulphur dispersion (80%)                                        | 3.75                     | 3                       |
| Zincoxide dispersion (50%)                                      | 12                       | 6                       |
| Zinc salt of phenylethyldithiocarbamic acid as dispersion (25%) | 4                        | 1                       |
| Paraphenyldiamine derivative (25%)                              | 8                        | 2                       |

After the second impregnation, the material was vulcanized by passing it over drying cylinders at a temperature of about 110° C. and final vulcanization and hardening of the synthetic resin components was accomplished by subsequent storing in a drying oven. Thereafter, the finally vulcanized and hardened material was thoroughly washed in washing machines whereby all water soluble components were dissolved out, leaving numerous fine and extra fine pores in the material. The material was then dried. It was characterized by extremely high porosity and absorptiveness. Generally, it had the properties of chamois leather, but, due to the presence of the phenol-formaldehyde resin, its abrasion resistance was substantially greater than that of natural leather.

Further experiments have shown that in some cases it is advantageous to introduce at least part of the synthetic resin condensates into the fibrous sheet material in a second impregnating stage following the impregnation of the sheet material with the elastic binders, such as natural or synthetic rubber. In these cases, the fiber fleece is treated in a first impregnating stage, preferably in the manner disclosed in the applicant's prior copending patent applications 262,941 and 262,942, with a dispersion or emulsion containing the film-forming binder and preferably such additional materials, as wetting agents, vulcanizing agents, antioxidants and the like, and the pre-impregnated sheet material thus obtained is then treated in a second impregnating stage with at least one synthetic resin precondensate, such as a precondensate of an aldehyde with phenols, urea or urea derivatives. Finally, the impregnated sheet material is subjected to a treatment suitable for the hardening of the synthetic resin condensate, for instance by heating in the presence of condensation catalysts.

This two-stage process has the advantage that it permits the introduction into the fibrous sheet material of such precondensates which are incompatible with one or more of the components of the binder liquids used for the principal impregnation of the fibrous material. Certain melamine resins are typical examples of this group of synthetic resins suitable for use in the second impreg-

nating stage of a two-stage impregnation. The secondary impregnation of the fibrous sheet material preimpregnated with film-forming binders may be carried out with emulsions, dispersions or solutions containing the synthetic resin precondensate in crystalloid-dispersed form, in colloid-dispersed form or in hetero-dispersed form. Such emulsions, dispersions or solutions may, in addition to the precondensates used, also contain catalysts capable of promoting the conversion of the precondensates to their insoluble final state. Suitable condensation catalysts are, for instance, ammonium salts, such as ammonium chloride, di-ammonium phosphate or propanol-aminehydrochloride, anorganic acids, such as hydrochloric acid or boric acid, anorganic bases, such as caustic soda solution or ammonia and organic bases such as, for instance, triethanolamine. The secondary impregnation may, for instance, be carried out with phenolic plastics in their soluble state, such as, for instance, the known precondensates of formaldehyde with urea or urea derivatives known under the trade names Ka 1525 or GFT 167, the urea precondensate known under the trade name Kaurit KW or the dicyandiamide known under the trade name Kaurit DD. Other suitable precondensates are known under the trade names Cassurit (trihydroxymethylmelamine), Lyofix MA (etherified trihydroxymethyl melamine), Lyofix CH (hexahydroxymethyl melamine) or Aerotex (etherified hydroxymethyl melamine).

It is recommended to use such precondensates which, after hardening, are resistant to organic solvents, as they are used in dry cleaning operations and which thus help to preserve the desired properties of the products, especially with regard to elasticity, springiness, feel, etc., even after several dry cleanings. Condensation products of melamine with formaldehyde or other aldehydes have been found to be particularly suitable for this purpose.

According to a further embodiment of the invention, the precondensates to be introduced into the fibrous sheet material are used partly in the first impregnating stage as components of the emulsions or dispersions containing the film-forming binder and partly in the second impregnating stage applied to the fibrous sheet material obtained from the first impregnating stage. It is possible to use in both impregnating stages precondensates of the same type, but, according to a preferred mode of operation, the first impregnating stage is carried out with emulsions or dispersions containing precondensates which are well compatible with the film-forming binders and other components of the binder liquids employed in this stage, while in the second impregnating stage (final impregnation) precondensates are used which are more or less incompatible with the components of the binder liquids used in the first impregnating stage. As mentioned before, melamine precondensates have been found to be particularly suitable for the second impregnating stage.

Generally, it is desirable to submit the fibrous sheet material after primary impregnation to a stabilizing and, if desired, vulcanizing treatment, for instance by heating, before carrying out the final impregnation by introducing the precondensates into the preimpregnated fibrous sheet material and subsequent hardening. Alternatively, the fibrous material leaving the first impregnating stage may be only lightly dried and submitted in this condition to the final impregnating treatment with synthetic resin precondensates. In the latter case, it is advisable to use for the second stage impregnation emulsions, dispersions or solutions which contain the synthetic resin precondensate in a relatively high concentration. The impregnating products are then subjected to a preferably intense drying and to a treatment, such as a heat treatment, which serves to harden the introduced precondensates. The hardening process may be carried out in such a manner that simultaneously the vulcanizable film-

forming binders introduced in the first impregnation stage are vulcanized. In this case, the second stage impregnation may be carried out with an emulsion, dispersion or solution containing, in addition to the synthetic resin precondensates and the condensation catalysts, also vulcanizing agents and possible vulcanization accelerators.

The second stage impregnation of the fibrous sheet material preimpregnated with film-forming binders can be carried out by saturating the material throughout with the emulsion, dispersion or solution of the synthetic resin precondensate followed by a suitable hardening step, if desired, after removal of excess precondensate liquid by squeezing out or the like. Alternatively, the second impregnating step may be so controlled that only one or both surface layers of the fibrous sheet material are impregnated to a desired depth with the synthetic resin precondensate liquid, for instance, by spraying or spreading of the latter upon one or both surfaces of the sheet material. This makes it possible to produce certain desired surface effects.

Finally, it has been found that in some cases it is advantageous to submit the fibrous sheet material into which, according to the present invention, synthetic resins have been introduced to an after-treatment with superheated steam, for instance in a drying room or under a press or on drying cylinders. Such treatment with superheated steam may, if desired, be utilized for the hardening of the synthetic resin condensate introduced into the fibrous material and/or for the vulcanization of the vulcanizable binders, such as rubber.

### Example 3

A fibrous fleece prepared and pre-stabilized by a unilateral surface treatment according to Example 1 was through impregnated in a first impregnating stage by passing it between a pair of rollers and pressing into the untreated surface thereof a stable flowable foam obtained from an aqueous dispersion containing the following solid ingredients:

Parts B. W.

|                                                                        |     |
|------------------------------------------------------------------------|-----|
| Butadiene-acrylonitrile polymer                                        | 100 |
| Sodiumsulphonate (dispersing agent)                                    | 27  |
| Sulphur                                                                | 3   |
| Active zincoxide                                                       | 5   |
| Vulkazit P extra N (Zinc salt of phenyl-diethyl-dithiocarbaminic acid) | 1   |

The preimpregnated sheet material was dried and then vulcanized at a temperature between about 70 and 130° C. Thereafter, the water soluble components can be eliminated by washing out, and the sheet material was dried again. Then, the material was treated in a second impregnating stage by introducing per 100 parts by weight of preimpregnated sheet material about 80 to 100 parts by weight of an aqueous solution containing per liter the following solid ingredients:

80 g. etherified trihydroxymethylmelamine (Lyofix MA)  
15 g. diammonium-phosphate  
15 g. dicyandiamide

The impregnated sheet material was pre-dried at about 80° C. and finally hardened for about ten minutes at 140° C. In a modification, pre-drying was omitted and the impregnated material was dried and hardened by heating it for twenty minutes to about 140° C.

### Example 4

A fiber fleece was prepared, surface stabilized and through impregnated in a first impregnating stage as described in Example 3, but in this case the foam used in the first impregnating stage was obtained from an

aqueous dispersion containing the following solid ingredients:

|                                                                        |      |
|------------------------------------------------------------------------|------|
| Parts B. W.                                                            |      |
| Butadiene-styrene polymer                                              | 50   |
| Butadiene-acrylonitrile polymer                                        | 50   |
| Phenolaldehyde precondensate                                           | 10.5 |
| Sodiumsulphonate                                                       | 20   |
| Sulphur                                                                | 3    |
| Active zincoxide                                                       | 5    |
| Vulkazit P extra N (Zinc salt of phenyl-diethyl-dithiocarbaminic acid) | 1.5  |
| Para-phenyldiamine derivative                                          | 2    |

After completion of the first stage impregnation, drying, vulcanizing and washing, the preimpregnated material was subjected to a second stage impregnation, as described in Example 3, with a solution containing per liter the following solid ingredients:

80 g. trihydroxymethylmelamine (Cassurit MKF)  
40 g. Kaurit DD (dicyandiamide precondensate)  
10 g. ammoniumchloride

In this case, drying and hardening were effected by heating the impregnated material for about 2½ minutes to 165°.

### Example 5

A surface stabilized fiber fleece was treated in a first impregnating stage, as described in Example 3, with a foam obtained from a dispersion of the following composition:

|                                                              | Liquid<br>Parts<br>B. W. | Solid<br>Parts<br>B. W. |
|--------------------------------------------------------------|--------------------------|-------------------------|
| Leguvol T 80 (polyester resin) dispersion                    | 27.1                     | 20.25                   |
| Emulphor FFO (30%) (alkyl-naphthylpolyglycol-ether) solution | 6                        | 1.8                     |
| Benzeneperoxide (Hardener-BPO paste) 90%                     | 0.72                     | 0.64                    |
| Nekal (alkyl-naphthalene-sulphonate)                         | 8                        | 8                       |
| Cobaltous chloride solution (20%)                            | 0.9                      | 0.18                    |
| Softened water                                               | 48.1                     |                         |

After drying, vulcanization and washing, the material was treated in a second impregnating stage with a solution containing per liter the following solid ingredients:

125 g. etherified hydroxymethylmelamine (Aerotex M3)  
15 g. of a mixture containing isopropanolamine hydrochloride (UTX)  
20 g. dicyandiamide

After drying, the product was in this case hardened under a pressure of 0.5 kg. per square centimeter at a temperature of 160° C. It was found that complete conversion of the synthetic resin precondensate to its insoluble state occurred in two to three seconds.

The process according to the present invention makes it possible to produce porous sheet material which, due to the increased condensation of the fiber material, have a relatively high specific weight. The hand, the springiness and other properties are improved. Moreover, the products obtained according to the present invention are characterized by particularly smooth surfaces, and high resistance to dry cleaning fluids.

We claim:

1. In the manufacture of porous sheet material similar to textile or leather and containing from about 25-65% by weight of rubber based on the combined weights of fibers and rubber, wherein a fleece of cardable polyposed fibers is impregnated with an aqueous dispersion of a rubber and the impregnated fleece is thereafter dried to deposit the rubber primarily at the crossing points of the fibers, the improvement which comprises introducing into the fibrous sheet material, in addition to the rubber, from 1 to 15 parts by weight per 100 parts by weight of rubber solids of a water-soluble condensation product of formaldehyde with a member of the group consisting of ureas, melamines and phenols, and there-

## 11

after converting said condensation product to water-insoluble form.

2. The process of claim 1, wherein the condensation product is employed in an amount ranging from 2 to 6 parts by weight per 100 parts by weight of rubber solids. 5

3. The process of claim 1, wherein the condensation product is at least partly included in the aqueous dispersion of the rubber solids.

4. The process of claim 3, wherein the aqueous dispersion of rubber solids and condensation product is applied as a foam. 10

5. The process of claim 1, wherein the rubber solids have a high Defo value and the condensation product is employed in an amount ranging from 1 to 2 parts by weight per 100 parts by weight of rubber solids. 15

6. The process of claim 1, wherein the rubber solids have a low Defo value and the condensation product is employed in an amount ranging from 6 to 8 parts by weight per 100 parts by weight of rubber solids.

7. The process of claim 1, wherein the condensation product is at least partly applied as an aqueous dispersion after drying of the sheet material following depositing of the rubber solids. 20

## 12

8. The process of claim 1, wherein the condensation product is a water-soluble melamine formaldehyde.

9. The process of claim 1, wherein the aqueous rubber dispersion also contains a vulcanizing agent and the sheet material is subjected to vulcanization prior to application of the water-soluble condensation product.

## References Cited in the file of this patent

## UNITED STATES PATENTS

|           |                          |               |
|-----------|--------------------------|---------------|
| 1,459,499 | Brown et al. -----       | June 19, 1923 |
| 1,766,817 | Friedlander et al. ----- | June 24, 1930 |
| 1,899,535 | Teague -----             | Feb. 28, 1933 |
| 1,936,999 | Teague -----             | Nov. 28, 1933 |
| 2,088,227 | Battye -----             | July 27, 1937 |
| 2,267,316 | Thompson et al. -----    | Dec. 23, 1941 |
| 2,424,923 | Edgar -----              | July 29, 1947 |
| 2,467,233 | Rust -----               | Apr. 12, 1949 |
| 2,536,050 | Fluck -----              | Jan. 2, 1951  |
| 2,563,897 | Wilson -----             | Aug. 14, 1951 |
| 2,716,617 | Auestu -----             | Aug. 30, 1955 |